# EUROPEAN PATENT SPECIFICATION

(11) **EP 0 986 089 B1**
(45) Date of publication and mention of the grant of the patent: **26.03.2008**
(21) Application number: 99117579.5
(22) Date of filing: 06.09.1999
(51) Int. Cl.: H01J 29/96, H01J 9/00, H01C 17/10, H01C 7/00, H01J 29/88

(54) **Field emission display including oxide resistor**
Feldemissionsanzeige mit Oxid-Widerstand
Panneau d'affichage à effet de champ avec une résistance d'oxyde

(30) Priority: 08.09.1998 JP 25355498
(43) Date of publication of application: 15.03.2000
(73) Proprietor: MATSUSHITA ELECTRIC INDUSTRIAL CO., LTD, Kadoma-shi, Osaka 571-8501 (JP)
(72) Inventor: Aoki, Masaki, Osaka, 562-0024 (JP); Ohtani, Mitsuhiro, Osaka, 590-0024 (JP); Suzuki, Shigeo, Osaka, 573-0093 (JP); Asida, Hideki, Osaka 571-0064 (JP)
(74) Representative: Kügele, Bernhard

(56) References cited:
- GB-A- 1 595 061
- GB-A- 2 028 576
- US-A- 4 527 147
- PATENT ABSTRACTS OF JAPAN vol. 1997, no. 12, 25 December 1997 (1997-12-25) & JP 09 204109 A (RICOH CO LTD), 5 August 1997 (1997-08-05)

## Description

### BACKGROUND OF THE INVENTION

### 1. FIELD OF THE INVENTION:

The present invention relates to a resistor having a high area resistance value usable in an image and video display device utilizing an electron source, for example, a cathode-ray tube (hereinafter, referred to as a "CRT") or a field emission display (hereinafter, referred to as an "FED"), a method for producing such a resistor, a cathode-ray tube including such a resistor, and an FED including such a resistor.

### 2. DESCRIPTION OF THE RELATED ART:

Figure **6** is a schematic cross-sectional view of a conventional CRT **600** used in a color display apparatus. As shown in Figure **6**, the CRT **600** includes a face plate **601** acting as a fluorescent screen and a neck **602**. The neck **602** accommodates a cathode **603** and an electronic lens system **607**. The electronic lens system **607** includes a triode section **604** and a main electronic lens section **605** formed of a plurality of metal cylinders **605A** and **605B**. The electronic lens system **607** is structured so as to project a crossover image of an electronic beam from the cathode section **603** on the face plate **601** using the main electronic lens section **605**. Reference numeral **606** represents a built-in division-type resistor.

In the electronic lens system **607** having such a structure, a diameter DS of a spot image on the face plate **601** is found by expression (1) using an electrooptic magnitude M and a spherical aberration coefficient CS0. $DS = [ ( M \times dx + \left(1/2\right) ⁢ M \times CS ⁢ 0 \times α ⁢ {0}^{3} ⁢ {)}^{2} + {DSC}^{2} ⁢ {]}^{1 / 2}$
where dx is a virtual crossover diameter, α0 is a divergence angle of the beam, and DSC is a divergence component of the beam caused by the repulsive effect of a spatial charge.

Recently, efforts have been made to minimize the spherical aberration coefficient CS0 of the main electronic lens section **605** in order to provide a high precision image by minimizing the spot diameter DS on the face plate **601**.

Japanese Laid-Open Publication No. 61-147442, for example, discloses a method for reducing the spherical aberration coefficient CS0 by a built-in division-type resistor. Japanese Laid-Open Publication Nos. 60-208027 and 2-276138, for example, each disclose a method for reducing the spherical aberration coefficient CS0 by forming a convergence electrode of a spiral resistor in the neck of the CRT instead of forming a convergence electrode of the main electronic lens including a plurality of metal cylinders.

The division-type resistor and the spiral resistor are formed in the following manner as described in, for example, Japanese Laid-Open Publication Nos. 61-224402 and 6-275211.

A film is formed of a stable suspension including ruthenium hydroxide (Ru(OH)₃) and glass particles and excluding an organic binder. The film is formed on an inner surface of a glass tube (formed of, for example, low melting point lead glass having a softening point of 640°C) by dipping. The film is dried, and then cut into a spiral pattern. Then, the film is baked at a temperature of 400°C to 600°C to form a resistor including ruthenium oxide (RuO₂).

Japanese Laid-Open Publication Nos. 61-147442, 55-14627 and 6-275211 disclose another resistor having a high area resistance value, which is formed of RuO₂ and high melting point glass particles.

The resistor formed of RuO₂ and glass particles is formed in a zigzag pattern on an alumina (e.g., Al₂O₃) substrate by screen printing. Such a resistor (referred to as a "glaze resistor") has a total resistance value of 300 MΩ to 1000 MΩ. The alumina used as the substrate has a thermal expansion coefficient of 75 x 10⁻⁷/°C and a melting point of 2,050°C. Since a CRT requires a resistor which is highly reliable against a high voltage of about 30 kV and an electronic beam, the resistor formed of RuO₂ and glass particles is formed by baking at a relatively high temperature of 750°C to 850°C.

Japanese Laid-Open Publication No. 9-293465, for example, discloses still another resistor formed of RuO₂ and low melting point glass. The low melting point glass is, for example, PbO-B₂O₃-SiO₂-based glass and includes PbO at 65% or more by weight. The softening point of the low melting point glass is about 600°C or less.

The above-described spiral or zigzag-pattern resistors are provided in the neck of the CRT in order to minimize the spot diameter on the fluorescent screen and the deflecting power. In addition, a double anode CRT is also developed in which the electronic lens system includes a high resistance layer in a funnel portion thereof.

A resistor used in the electronic lens system of the CRT provides a potential distribution between the anode electrode and a focus electrode, and thus needs to have a sufficiently high area resistance value of 1 GΩ/□ to 100 GΩ/□ (i.e., about 10⁹ Ω/□ to about 10¹¹ Ω/□) in order to prevent a current flow sufficiently to avoid sparking and arc discharge.

Displays utilizing an electron source, such as an FED, also require a high area resistance value provided between an anode and a cathode.

According to the method described in Japanese Laid-Open Publication Nos. 61-224402 and 6-275211, Ru(OH)₃, which is an insulating substance, is thermally decomposed while being baked at a temperature of 400°C to 600°C. By such thermal decomposition, RuO₂, which is a conductive substance, is deposited, and the low melting point glass flows. As a result, fine particles of RuO₂ having a diameter of 0.01 to 0.03 µm are deposited around the glass particles, which form a resistor.

Such a method has the following problems in obtaining a high resistance value of 5 GΩ to 20 GΩ (area resistance value: 1 MΩ/□ to 4 MΩ/□): (i) the dependency of the area resistance value on the baking temperature increases (i.e., the area resistance value significantly changes when the baking temperature slightly changes): (ii) the temperature coefficient of resistance value (TCR) is increased in a negative direction; and (iii) the load characteristic over a long period of time is inferior. The expression "/□" refers to "per unit area".

The method described in Japanese Laid-Open Publication Nos. 55-14527, 61-147442 and 6-275211 has a problem in that the resultant resistor cannot be formed on an inner surface of the low melting point glass (having a softening point of 640°C) used for the CRT due to the high baking temperature of 750°C to 850°C.

According to the method described in Japanese Laid-Open Publication No. 7-309282, the resistor can be formed on an inner surface of the CRT at a low temperature of 440°C to 520°C. However, the resistor formed by this method has problems in that (i) the area resistance value significantly changes in accordance with the load characteristic (against application of a voltage of 30 kV at 70°C at 10⁻⁷ Torr) in the vacuum over a long period of time (5,000 hours); and (ii) the spot diameter on the fluorescent screen is increased due to the load since the TCR is negative.

A tungsten (W)-aluminium oxide-based cermet resistor having a high area resistance value has been developed for use in the electronic tube (see, for example, Japanese Publication for Opposition No. 56-15712). Such a resistor has problems in that (i) a high area resistance value of 10⁹ Ω/□ or more is not obtained; and (ii) the TCR is negative and the absolute value thereof is excessively large.

A resistor having an area resistance value of 1 GΩ/ □ to 100 GΩ/□ does not need to be shaped into a spiral or zigzag pattern, for use in a CRT. However, the conventional resistive materials have an area resistance value of 1 MΩ/ □ to 100 MΩ/□. Since such a range of area resistance values is not sufficiently high, the resistor needs to be shaped into a spiral or zigzag pattern.

Attempts have been made to produce an electronic lens system using a high resistance ceramic cylinder without shaping the resistor into a spiral or zigzag pattern (see, for example, Japanese Laid-Open Publication No. 6-275211 and the Proceedings of the 14th International Display Research Conference, pp. 229 to 232 (1994)).

The resistive materials used for this type of electronic lens system include forsterite (2MgO·SiO₂) -based and Al₂O₃-MnO₂-Fe₂O₃-Nb₂O₃-based materials. The specific resistance value of these materials is 10¹¹ Ωcm (resistance value: 2.4 GΩ to 240 GΩ). However, it has been pointed out that when the power consumption of a display apparatus, for example, a TV is increased by the negative TCR, the current flowing in the resistive material rapidly increases and possibly thermal runaway occurs.

Reference may be made to WO 98/03986 which discloses the pre-characterizing features of the present invention. Reference may also be made to GB 1595061, US 5675212 and US 5663608

### SUMMARY OF THE INVENTION

The present invention is defined in the claims.

The present inventors have found that, in various forms: (i) an appropriate metal conductive oxide and insulating oxide at an appropriate ratio can be produced for a field emission display by a flame spraying method and can yield a resistor having a high area resistance value of about 1 GΩ/□ to about 100 GΩ/□ is produced: (ii) the resultant resistor has a superior overtime load characteristic to the conventional resistors; and (iii) the TCR of the resultant resistor is small and stable.

Such a resistor does not need to be shaped into a spiral or zigzag pattern.

Advantages of the invention include the ability to provide a field emission display comprising: (1) a resistor having a satisfactory high area resistance value produced without baking; (2) a resistor having a satisfactory high load characteristic over a long period of time in vacuum: (3) a reliable resistor having a small TCR.

These and other advantages of the present invention will become apparent to those skilled in the art upon reading and understanding the following detailed description with reference to the accompanying figures.

### BRIEF DESCRIPTION OF THE DRAWINGS

Figure **1A** is a schematic view of a plasma flame-spraying apparatus used for producing a resistor in a first example ;
Figure **1B** is a flowchart illustrating a method for producing the resistor shown in Figure **1A**;
Figure **2** is a schematic cross-sectional view of a CRT including the resistor shown in Figure **1A**;
Figure **3A** is a schematic view of a laser flame-spraying apparatus used for producing a resistor in a second example
Figure **3B** is a flowchart illustrating a method for producing the resistor shown in Figure **3A**;
Figure **4** is a schematic cross-sectional view of a CRT including the resistor shown in Figure **3A**;
Figure **5A** is an isometric view of an FED in a third example according to the present invention;
Figure **5B** is a cross-sectional view of the FED shown in Figure 5A taken along surface **A**; and
Figure **6** is a schematic cross-sectional view of a conventional CRT.

### DESCRIPTION OF THE EMBODIMENTS

Hereinafter, the present invention will be described by way of illustrative examples with reference to the accompanying drawings.

### (Example 1)

A resistor produced by a plasma flame-spraying method in a first example usable with, but not forming part of, the present invention will be described with reference to Figures **1A**, **1B** and **2**.

Figure **1A** is a schematic view of a plasma flame-spraying apparatus **100** used for producing a resistor in the first example. Figure **1B** is a flowchart illustrating a method for producing the resistor in the first example.

As shown in Figure **1A**, the plasma flame-spraying apparatus **100** includes a negative electrode 101, a positive electrode **102**, a power supply **103**, a spray nozzle **107**, and a powder supply port **109** for supplying a resistive material **108**. Reference numeral **104** represents a DC arc, and reference numeral **105** represents operation gas. Reference numeral **106** represents an arc plasma jet **106**. Reference numeral **110** represents an alumina (e.g., Al₂O₃) substrate, and reference numeral **111** represents an electrode (for example, focus electrode and anode electrode). Reference numeral **112** represents a resistor produced by the plasma flame-spraying apparatus **100**. A glass substrate may be used instead of the alumina substrate **110**.

With reference to Figure **1B**, a method for producing the resistor **112** will be described. Refer to Figure **1A** for the reference numeral of each element.

In step S101, a silver paste, for example, is screen-printed on the alumina substrate **110** and then baked, thereby forming the electrodes **111**.

Then, in step S102, an electric field is applied between the negative electrode **101** and the positive electrode **102** using the power supply **103** to generate the DC arc **104**. The operation gas **105** (e.g., argon-hydrogen mixture gas or nitrogen-hydrogen mixture gas) is caused to flow along a surface of the negative electrode **101** to generate the arc plasma jet **106**.

In step S103, the resistive material **108** including, for example, a mixture powder including TiO at about 30% by weight and Al₂O₃ at about 70% by weight is supplied from the power supply port **109**. While the spray nozzle **107** is moved toward the alumina substrate **110**, the resistive material **108** is flame-sprayed toward the alumina substrate **110** to a thickness of about 20 µm, thereby forming the resistor **112** on the alumina substrate **110**. In the case where the resistive material **108** needs to be flame-sprayed under a low pressure atmosphere of about 0.1 to about 10 Torr, the plasma flame-spraying apparatus **100** is entirely accommodated in a low pressure chamber before the production.

Then, Al₂O₃ is sprayed toward the resistor **112** to a thickness of about 40 µm, thereby forming a protective film (not shown). Al₂O₃ is not sprayed to the electrodes **111**. Thus, a resistor section **113** including the TiO-Al₂O₃-based resistor 112, the alumina substrate **110** and the electrodes **111** is formed.

The TiO- Al₂O₃-based resistor 112, which is produced without a baking process, has a high area resistance value of about 1 GΩ/□ or more and also a satisfactory heat-resistant load characteristic as described below. Furthermore, the TiO-Al₂O₃-based resistor **112** has a positive and stable TCR.

Figure **2** is a schematic cross-sectional view of a CRT **200** not forming part of the invention, and including the resistor section **113**. Identical elements previously discussed with respect to Figure **6** bear identical reference numerals and the descriptions thereof will be omitted.

The resistor section **113**, as described above with reference to Figure **1A**, includes the TiO-Al₂O₃-based resistor **112**, the alumina substrate **110** and the electrodes **111**.

The CRT **200** including the TiO-Al₂O₃-based resistor **112** enjoys the above-described advantages of the TiO-Al₂O₃-based resistor **112**.

The present invention is not limited to the TiO Al₂O₃-based resistor **112**. Usable instead of TiO are both or either of a metal conductive oxide or a transition metal material. Usable instead of Al₂O₃ is an insulating oxide.

### (Example 2)

A resistor produced by a laser flame-spraying method in a second example usable with, but not forming part of the present invention will be described with reference to Figures **3A**, **3B** and **4**.

Figure **3A** is a schematic view of a laser flame-spraying apparatus **300** used for producing a resistor in the second example. Figure **3B** is a flowchart illustrating a method for producing the resistor in the second example.

As shown in Figure **3A**, the laser flame-spraying apparatus **300** includes a spray nozzle **201**, a powder supply port **202** for supplying a resistive material (not shown), and a laser light collection lens system **204**. The powder supply port **202** is formed so as to run throughout the spray nozzle **201**. Reference numeral **203** represents laser light. Reference numeral **205** represents a glass tube of a CRT, and reference numeral **206** represents an electrode. Reference numeral **207** represents a resistor produced by the laser flame-spraying apparatus **300**.

With reference to Figure **3B**, a method for producing the resistor **207** will be described. Refer to Figure **3A** for the reference numeral of each element.

In step S301, the electrodes **206** (for example, anode electrode and focus electrode) are formed on an inner surface of the glass tube **205** of the CRT. The electrodes **206** can be formed of the same material and in the same manner as those of the electrodes **111** described in the first example.

Then, in step S302, the laser light **203** is collected by the laser light collection lens system **204**. In step S303, a resistive material (not shown) including, for example, a mixture powder including TiO at about 10% by weight and Al₂O₃ at about 90% by weight is supplied from the power supply port **202**. While the spray nozzle **201** is moved toward the glass tube **205**, the resistive material is flame-sprayed toward the glass tube **205** to a thickness of about 20 µm, thereby forming resistor **207** on the glass tube **205.** Since the resistor **207** is formed on the inner surface of the glass tube **205**, it is not necessary to form a protective film as is necessary in the first example.

The TiO-Al₂O₃-based resistor **207**, which is produced without a baking process, has a high area resistance value of about 1 GΩ/□ and also a satisfactory heat-resistant load characteristic as described below. Furthermore, the TiO-Al₂O₃-based resistor **207** has a positive and stable TCR.

Figure **4** is a schematic cross-sectional view of a CRT **400** not forming part of the present invention, and including the TiO-Al₂O₃-based resistor **207.**

The CRT **400** includes the TiO-Al₂O₃-based resistor **207** provided on the inner surface of the glass tube **205**, and the electrodes **206**. An inner surface **401** of the CRT **400** is coated with a paste of graphite, RuO₂ or the like.

The CRT **400** including the TiO-Al₂O₃-based resistor **207** enjoys the above-described advantages of the TiO-Al₂O₃-based resistor 207.

The technique is not limited to the TiO-Al₂O₃-based resistor **207**. Usable instead of TiO are both or either of a metal conductive oxide or a transition metal material. Usable instead of Al₂O₃ is an insulating oxide.

### (Example 3)

In a third example, an FED **500** including a resistor according the present invention will be described with reference to Figure **5A** and **5B**.

Figure **5A** is an isometric view of the FED **500**. Figure **5B** is a cross-sectional view of the FED **500** taken along surface **A** in Figure **5A**.

As shown in Figures **5A** and **5B**, the FED **500** includes an anode **501**, a cathode **502**, an FED array **503** provided on an inner surface of the cathode **502**, a cathode drawing electrode **504** connected to the cathode **502**, an anode drawing electrode **505** connected to the anode **501**, a fluorescent body **508** provided on an inner surface of the anode **501**, and a power supply **507**.

Supports **506** are provided between the anode **501** and the cathode **502** for preventing the anode **501** and the cathode **502** from contacting each other in vacuum. The supports **506** are formed of glass, alumina or any other insulating material.

The supports **506** are covered with the TiO-Al₂O₃-based resistor **112** described in the first example or the TiO-Al₂O₃-based resistor **207** in the second example.

Without such a resistor, the following inconvenience occurs. When a high voltage of several kilovolts to several tens of kilovolts is applied between the anode drawing electrode **504** and the cathode drawing electrode **505**, electrons are accumulated in the supports **506** since the supports **506** are formed of an insulating material. When the electrons are accumulated in the supports **506**, arc or spark is generated from the supports **506**. As a result, an image on a screen of the FED **500** is disturbed or the fluorescent body **508** is damaged.

In the FED **500** including the above-described resistor, the electrons accumulated in the supports **506** are removed by causing a slight amount of current to flow in the supports **506**. Accordingly, the electrons are not accumulated, which prevents generation of arc or spark from the supports **506** or damages on the fluorescent body **508**.

### [Specific Examples]

TiO and Al₂O₃-based resistors are produced with various ratios of TiO and Al₂O₃. Resistors including both or either of a metal conductive oxide or a transition metal material (e.g., ReO₃, IrO₂, MoO₂, WO₂, RuO₂, LaTiO₃, or TiO₂₋ₓ (0<x<1)), and an insulating oxide (e.g., SiO₂, ZrO₂, or MgO) are also produced with various ratios.

The resistors are produced by a plasma flame-spraying method or a laser flame-spraying method.

The resultant resistors are each attached to an electronic gun of the CRT **200** (Figure **2**) or the CRT **400** (Figure **4**), or provided on the supports **506** of the FED **500** (Figures **5A** and **5B**).

An accelerated test of the CRT **200** can be performed by applying a voltage of about 30 kV to about 40 kV to the anode electrode (e.g., electrode 111 in Figure **1A**) and applying a voltage of about 5 kV to about 10 kV to the focus electrode (e.g., electrode **111** in Figure **1A**). In this example, a voltage of about 30 kV is applied to the anode electrode for about 5,000 hours for testing the life of the CRT **200** (test of actual life). A voltage of about 45 kV is applied to the anode electrode for about 10 hours for testing the life of the CRT **200** when an excessive load is applied (test of life against short-time application of excessive load).

An accelerated test of the CRT **400** can be performed by applying a voltage of about 10 kV to about 30 kV between the electrodes **206**. In this example, a voltage of about 30 kV is applied between the electrodes **206** for about 5,000 hours for testing the life of the CRT **400** (test of actual life). A voltage of about 45 kV is applied to the anode between the electrodes **206** for about 10 hours for testing the life of the CRT **400** when an excessive load is applied (test of life against short-time application of excessive load).

An accelerated test of the FED **500** is performed by applying a voltage of about 15 kV between the anode drawing electrode **504** and the cathode drawing electrode **505**. An area resistance value, temperature characteristic of resistance value (TCR), and overtime change in the area resistance value, and the like are evaluated.

The conditions for producing the resistors are shown in Tables 1 through 4. The evaluation results are shown in Tables 5 and 6. Samples 15 through 19 in Table 2 are

**Table 1**

| Sample | Materials and ratio (% by weight) | | | | Method for formation | Substrate | Use | Pattern of resistor |
|---|---|---|---|---|---|---|---|---|
| | Metal conductive oxide | | Insulating oxide film | | | | | |
| 1 | TiO | (30) | Al2O₃ | (70) | Plasma flame-spraying (Ar-H₂ gas) | Alumina (Al₂O₃) | Division-type resistor | Plain |
| 2 | TiO | (5) | Al₂O₃ | (95) | Plasma flame-spraying (N₂-H₂ gas) | Alumina (Al₂O₃) | Division-type resistor | Plain |
| 3 | TiO | 3) | Al₂O₃ | (97) | Laser flame-spraying | Alumina (Al₂O₃) | Division-type resistor | Plain |
| 4 | ReO₃ | (5) | SiO₂ | (95) | Laser flame-spraying | Alumina (Al₂O₃) | Division-type resistor | Plain |
| 5 | IrO₂ | (5) | ZrO₂ | (95) | Plasma flame-spraying (N₂-H₂ gas) | Alumina (Al₂O₃) | Division-type resistor | Plain |
| 6 | RuO₂ | (3) | MgO | (97) | Plasma flame-spraying (Ar-H₂ gas) | Alumina (Al₂O₃) | Division-type resistor | Plain |
| 7 | VO | (5) | Al₂O₃ | (95) | Plasma flame-spraying (Ar-H₂ gas) | Alumina (Al₂O₃) | Division-type resistor | Plain |
| 8 | RhO₂ | (4) | Al₂O₃ | (96) | Laser flame-spraying | CRT glass tube | Inner surface of CRT | Plain |
| 9 | La TiO₃ | (5) | Al₂O₃ | (95) | Plasma flame-spraying (N₂-H₂ gas) | CRT glass tube | Inner surface of CRT | Plain |
| 10 | SrRuO₃ | (5) | Al2 O₃ | (95) | Plasma flame-spraying (N₂-H₂ gas) | CRT glass tube | Inner surface of CRT | Plain |

**Table 2**

| Sample | Materials and ratio (% by weight) | | | | Method for film formation | Substrate | Use | Pattern of resistor |
|---|---|---|---|---|---|---|---|---|
| | Metal conductive oxide (Except for samples 17, 18 and 19) | | Insulating oxide | | | | | |
| 11 | MoO₂ | (5) | Al₂O₃ | (95) | Plasma flame-spraying (N₂-H₂ gas) | Alumina (Al₂O₃) | Division-type resistor | Plain |
| 12 | WO₂ | (5) | Al₂O₃ | (95) | Plasma flame-spraying (N₂-H₂ gas) | Alumina (Al₂O₃) | Division-type resistor | Plain |
| 13 | NbO | (5) | SiO₂ | (95) | Plasma flame-spraying (N₂-H₂ gas) | Alumina (Al₂O₃) | Division-type resistor | Plain |
| 14 | OsO₂ | (5) | SiO₂ | (95) | Plasma flame-spraying (N₂-H₂ gas) | Alumina (Al₂O₃) | Division-type resistor | Plain |
| 15* | RuO₂ | (3) | Lead-based glass (PbO-SiO₂-B₂O₃-Al₂O₃) | (97) | Paste is screen-printed and baked at 800°C | Alumina (Al₂O₃) | Division-type resistor | Zigzag |
| 16* | Ru O₂ | (PbO-SiO₂-B2O₃-Al₂O3) | Lead-based glass PbO-SiO₂-B₂O₃-Al₂O₃) | (97) | Paste is screen-printed and baked at 450 °C | CRT glass tube | Inner surface of CRT | Zigzag |
| 17* | Al₂O₃-MnO₂-Fe₂O₃-Nb₂O₃-based ceramic | | | | Baked | Cylinder in CRT | | Zigzag |
| 18* | W | (20) | Al₂O₃ | (80) | Sputtered and baked at 850°C in vacuum | Alumina (Al₂O₃) | Division-type resistor | Plain |
| 19* | Mo | (20) | Al₂O₃ | (80) | Sputtered and baked at 850°C in vacuum | Alumina (Al₂O₃) | Division-type resistor | Plain |

| | | | | | | | | |
|---|---|---|---|---|---|---|---|---|
| * Samples 15 through 19: conventional resistors | | | | | | | | |

**Table 3**

| Sample | Materials and ratio (% by weight ) | | | | Method for film formation | Substrate | Use | Pattern of resistor |
|---|---|---|---|---|---|---|---|---|
| | Metal conductive oxide or transition metal material | | Insulating oxide | | | | | |
| 20 | TiO | (10) | Al₂O₃ | (90) | Plasma flame-spraying (Ar-H₂ gas) | Glass support in FED | Charge prevention (Arc and spark prevention) | Plain |
| 21 | TiO_{1.5} | (5) | Al₂O₃ | (95) | Plasma flame-spraying (N₂-H₂ gas) | Glass support in FED | Charge prevention (Arc and spark prevention) | Plain |
| 22 | Ti O_{1.2} | (3) | Al₂O₃ | (97) | Laser flame-spraying | Glass support in FED | Charge prevention (Arc and spark prevention) | Plain |
| 23 | ReO₃ | (5) | SiO₂ | (95) | Laser flame-spraying | glass support in FED | Charge prevention (Arc and spark prevention) | Plain |
| 24 | IrO₂ | (5) | ZrO₂ | (95) | Plasma flame-spraying (N₂-H₂ gas) | Glass support in FED | Charge prevention (Arc and spark prevention) | Plain |
| 25 | RuO₂ | (5) | mgO | (95) | Plasma flame-spraying (Ar-H₂ gas) | Glass support in FED | Charge prevention (Arc and-spark prevention) | Plain |
| 26 | VO | (10) | Al₂O₃ | (90) | Plasma flame-spraying (Ar-H₂ gas) | Glass. support in FED | Charge prevention (Arc and spark prevention) | Plain |

**Table 4**

| Sample | Materials and ratio (% by weight) | | | | Method for film formation | Substrate | Use | Pattern of resistor |
|---|---|---|---|---|---|---|---|---|
| | Metal conductive oxide or transition metal material | | Insulating oxide | | | | | |
| 27 | RhO₂ | (5) | Al₂O₃ | (95) | Laser flame-spraying | CRT glass tube | Inner surface of CRT | Plain |
| 28 | Ti | (5) | Al₂O₃ | (95) | Plasma flame-Spraying (N₂-H₂ gas) | CRT glass tube | Inner surface of CRT | Plain |
| 29 | Re | (5) | Al₂O₃ | (95) | Plasma flame-spraying (N₂-H₂ gas) | CRT glass tube | Inner surface of CRT | Plain |
| 30 | V | (5) | Al₂O₃ | (95) | Plasma flame-spraying (N₂-H₂ gas) | Glass support in FED | Charge prevention (Arc and spark prevention) | Plain |
| 31 | Nb | (5) | Al₂O₃ | (95) | Plasma flame-spraying (N₂-H₂ gas) | Glass support in FED | Charge prevention (Arc and spark prevention) | Plain |

**Table 5**

| Sample | Thickness | Area resistance value | Temperature characteristic of resistance value (TCR) (PPm/°C) | 10⁻⁷ Torr 70 °C 30kV: change in area resistance value after 5000 hrs. | 45kV: change in area resistance value after 10 hrs. |
|---|---|---|---|---|---|
| 1 | 20 µm | 1 GΩ | -150 | 0.3 % | -0.5 % |
| 2 | 20 µm | 10 GΩ | -350 | 0.25 % | -0.5 % |
| 3 | 35 µm | 100 GΩ | -300 | 0.2 % | -0.6 % |
| 4 | 40 µm | 15 GΩ | +1500 | 0.5% | -0.7 % |
| 5 | 30 µm | 50 GΩ | +1500 | 0.3 % | -0.8 % |
| 6 | 30 µm | 1 GΩ | +35 | 0.3% | -0.7 % |
| 7 | 30 µm | 5 GΩ | -45 | 0.5 % | -1.2 % |
| 8 | 30µm | 3GΩ | +200 | 0.4% | -1.0% |
| 9 | 30µm | 10 GΩ | -30 | 0.5% | -1.5% |
| 10 | 30 µm | 4 GΩ | -55 | 0.3% | -1.3% |
| 11 | 30 µm | 1GΩ | -20 | -0.8% | -1.2% |
| 12 | 30 µm | 2 GΩ | -35 | -0.7% | -1.5% |
| 13 | 30µm | 10 GΩ | -18 | -0.5% | -1.0% |
| 14 | 30 µm | 3GΩ | +1500 | +0.8% | -0.8% |
| 15 | 5µm | 1 GΩ | +340 | -1.2% | -15 % |
| 16 | 5 µm | 10 GΩ | +420 | -1.5% | -20% |

**Table 6**

| Sample | Thickness | Area resistance value | Temperature characteristic of resistance value (TCR) (PPM/° C) | 10⁻⁷ Torr 70 °C 30kV: change in area resistance value after 5000 hrs. | 45kV: change in area resistance value after 10 hrs. |
|---|---|---|---|---|---|
| 17 | 5 µm | 100 GΩ | + 1500 | 5.2 % | -15 % |
| 18 | 5 µm | 1 GΩ | +11000 | -15 % | Cracks in substrate |
| 19 | 5 µm | 2 GΩ | +10000 | -19% | Cracks in substrate |
| 20 | 20 µm | 8 GΩ | +50 | 0.3% | -0.6% |
| 21 | 20 µm | 10 GΩ | -103 | -0.35% | -0.5 % |
| 22 | 20 µm | 100 GΩ | -305 | -0.3% | -0.6% |
| 23 | 20 µm | 5 GΩ | + 105 | -0.5 % | -0.8 % |
| 24 | 20 µm | 10GΩ | + 10 | -0.2 % | -0.7% |
| 25 | 20 µm | 15 GΩ | +10 | 0.3% | -1.0% |
| 26 | 20µm | 150 GΩ | -1500 | -0.8 % | -1.2% |
| 27 | 20 µm | 18GΩ | -150 | -0.3% | -1.0% |
| 28 | 20 µm | 52 GΩ | -450 | -0.5 % | -1.5% |
| 29 | 20 µm | 30 GΩ | -520 | -0.7% | -1.3 % |
| 30 | 20 µm | 180 GΩ | -1550 | -0.8 % | - 1.2 % |
| 31 | 20 µm | 205 GΩ | -1630 | -0.9% | -1.2% |

It is appreciated from Tables 1 through 6 that compared to a conventional RuO₂-glass-based resistor, a conventional ceramic resistor, or a conventional cermet resistor including Mo (molybdenum) or W (tungsten) and an insulating oxide, the resistors including both or either of a metal conductive oxide or a transition metal material, and an insulating oxide have a higher area resistance value, exhibit a smaller change in the TCR, and change less in the area resistance value against a load at an area identical resistance value (i.e., have a higher durability against application of a high voltage).

When a high load of about 45 kV is applied, the conventional resistors are significantly damaged.

As described above, a resistor may be formed of a mixture of both or either of a metal conductive oxide or a transition metal material, and an insulating oxide; and is formed on alumina or glass by a plasma flame-spraying method or a laser flame-spraying method. Such a resistor has a sufficiently high area resistance value and is obtained without a baking process.

Since the particles of the metal conductive oxide or the transition metal material are dispersed among the particles of the insulating oxide, the resistor formed of the above-described mixture has a sufficiently high area resistance value.

The resistor according to the above technique is stable due to a superior load characteristic in vacuum and a small TCR.

The metal conductive oxides usable in the resistor include, for example, titanium oxide, rhenium oxide, iridium oxide, ruthenium oxide, vanadium oxide, rhodium oxide, osmium oxide, lanthanum titanate, SrRuO₃, molybdenum oxide, tungsten oxide, and niobium oxide. These oxides can be used independently or in combination of two or more.

Preferably, T10, ReO₃, IrO₂, RuO₂, VO, RhO₂, OsO₂, LaTiO₃, SrRuO₃, MoO₂, WO₂, and NbO are used.

The transition metal materials usable in the resistor include, for example, titanium, rhenium, vanadium niobium. These materials can be used independently or in combination of two or more.

The insulating oxides usable in the resistor include, for example, alumina, silicon oxide, zirconium oxide, and magnesium oxide. These materials can be used independently or in combination of two or more.

Preferably, Al₂O₃, SiO₂, ZrO₂, and MgO are used.

Various other modifications will be apparent to and can be readily made by those skilled in the art without departing from the scope of this invention.

## Claims

1. A field emission display, comprising:
an anode (501);
a cathode (502); and
a resistor (112) provided between the anode (501) and the cathode (502),
wherein:
the resistor (112) includes a mixture of a metal conductive oxide with an insulating oxide, **characterized in that**:
the metal conductive oxide is at least one material selected from the group consisting of TiO, rhenium oxide, iridium oxide, ruthenium oxide, rhodium oxide, osmium oxide, lanthanum titanate, SrRuO₃, molybdenum oxide, tungsten oxide, and niobium oxide, and
the resistor (112) has an area resistance value of at least about 1 GΩ/□.

2. A field emission display according to claim 1, further comprising a support (506) provided between the anode (501) and the cathode (502), wherein the support (506) is covered with the resistor (112).

3. A field emission display according to claim 2, wherein the support (506) includes at least one of glass and alumina.

4. A field emission display according to claim 1, wherein the insulating oxide is at least one material selected from the group consisting of alumina, silicon oxide, zirconium oxide, and magnesium oxide.

5. A field emission display according to claim 1, wherein the insulating oxide is at least one material selected from the group consisting of Al₂O₃, SiO₂, ZrO₂, and MgO.

6. A field emission display according to claim 1, wherein the metal conductive oxide is TiO, and the insulating oxide is Al₂O₃.

## Patentansprüche

1. Feldemissionsanzeige, die umfasst:
eine Anode (501);
eine Katode (502); und
einen Widerstand (112), der zwischen der Anode (501) und der Katode (502) vorgesehen ist,
wobei:
der Widerstand (112) ein Gemisch aus einem leitenden Metalloxid und einem isolierenden Oxid enthält, **dadurch gekennzeichnet, dass**:
das leitende Metalloxid wenigstens ein Material ist, das aus der Gruppe ausgewählt ist, die aus TiO, Rheniumoxid, Iridiumoxid, Rutheniumoxid, Rhodiumoxid, Osmiumoxid, Lanthantitanat, SrRuO₃, Molybdänoxid, Wolframoxid und Nioboxid besteht, und
der Widerstand (112) einen Flächenwiderstandswert von wenigstens etwa 1 GΩ/□ besitzt.

2. Feldemissionsanzeige nach Anspruch 1, die ferner einen Träger (506) umfasst, der zwischen der Anode (501) und der Katode (502) vorgesehen ist, wobei der Träger (506) mit dem Widerstand (112) abgedeckt ist.

3. Feldemissionsanzeige nach Anspruch 2, wobei der Träger (506) Glas und/oder Aluminiumoxid enthält.

4. Feldemissionsanzeige nach Anspruch 1, wobei das isolierende Oxid wenigstens ein Material ist, das aus der Gruppe ausgewählt ist, die aus Aluminiumoxid, Siliciumoxid, Zirkonoxid und Magnesiumoxid besteht.

5. Feldemissionsanzeige nach Anspruch 1, wobei das isolierende Oxid wenigstens ein Material ist, das aus der Gruppe ausgewählt ist, die aus Al₂O₃, SiO₂, ZrO₂ und MgO besteht.

6. Feldemissionsanzeige nach Anspruch 1, wobei das leitende Metalloxid TiO ist und das isolierende Oxid Al₂O₃ ist.

## Revendications

1. Ecran à émission de champ, comprenant :
une anode (501) ;
une cathode (502) ; et
une résistance (112) disposée entre l'anode (501) et la cathode (502),
dans lequel :
la résistance (112) comprend un mélange d'un oxyde métallique conducteur avec un oxyde isolant, **caractérisé en ce que** :
l'oxyde métallique conducteur est au moins un matériau choisi dans le groupe constitué par le TiO, l'oxyde de rhénium, l'oxyde d'iridium, l'oxyde de ruthénium, l'oxyde de rhodium, l'oxyde d'osmium, le titanate de lanthane, le SrRuO₃, l'oxyde de molybdène, l'oxyde de tungstène, et l'oxyde de niobium, et
la résistance (112) a une valeur de résistance de surface d'au moins environ 1 GΩ/□.

2. Ecran à émission de champ selon la revendication 1, comprenant en outre un support (506) disposé entre l'anode (501) et la cathode (502), dans lequel le support (506) est recouvert avec la résistance (112).

3. Ecran à émission de champ selon la revendication 2, dans lequel le support (506) comprend au moins l'un parmi le verre et l'alumine.

4. Ecran à émission de champ selon la revendication 1, dans lequel l'oxyde isolant est au moins un matériau choisi dans le groupe constitué par l'alumine, l'oxyde de silicium, l'oxyde de zirconium, et l'oxyde de magnésium.

5. Ecran à émission de champ selon la revendication 2, dans lequel l'oxyde isolant est au moins un matériau choisi dans le groupe constitué par l'Al₂O₃, le SiO₂, le ZrO₂, et le MgO.

6. Ecran à émission de champ selon la revendication 1, dans lequel l'oxyde métallique conducteur est le TiO, et l'oxyde isolant est l'Al₂O₃.
